

## UNITED STATES PATENT OFFICE

2,131,520

## ALUMINUM ALLOY

Joseph A. Nock, Jr., Tarentum, Pa., assignor to  
Aluminum Company of America, Pittsburgh,  
Pa., a corporation of Pennsylvania

No Drawing. Application September 16, 1936,  
Serial No. 101,132

7 Claims. (Cl. 148—32)

This invention relates to aluminum base alloys, especially those containing from 2 to 12 per cent copper, 0.1 to 2 per cent silicon, and 0.005 to 0.1 per cent tin. These alloys develop exceptionally desirable physical properties when subjected to the well known solution and precipitation hardening thermal treatments. In order to obtain the best combination of high physical properties and resistance to corrosion, it has been found 5 that the alloys must be practically free from any magnesium impurity. In commercial practice not more than 0.01 per cent is generally permitted, and less than 0.005 per cent is preferred. Such requirements have necessitated the use of 10 virgin aluminum, or carefully selected scrap metal containing a minimum of magnesium impurity, and the exercise of particular care in preventing contamination from the melting furnace hearth and other containers of the molten metal. Such 15 precautions obviously add to the cost of producing the alloys, as well as restricting the supply of metal which can be drawn upon for this purpose. It is therefore highly desirable both to utilize metal having a larger magnesium impurity content and yet to overcome the deleterious 20 effects of this impurity, particularly if it happens to exceed the specified limits. My invention is directed to achieving the foregoing improvements, and it is primarily concerned with providing a 25 means of improving the resistance to corrosion of these alloys.

A means of suppressing the harmful effect of magnesium impurity in aluminum-copper-tin alloys of the type referred to hereinabove, is 30 described in formerly co-pending application, Serial No. 750,016, now issued as Patent No. 2,063,942. It is pointed out in that application that the addition of from 0.05 to 0.15 per cent cadmium to the alloys containing between 0.005 35 and 0.03 per cent magnesium, in the ratio of 5 to 1, improves the resistance to corrosion as well as increasing the strength of such alloys. I have now found that the resistance to corrosion can be even further improved by the addition of 0.1 to 3 per cent zinc along with the cadmium in the aforesaid amounts and ratio. The zinc addition is of particular benefit where the alloys are subjected to severe corrosive conditions while under stress. To distinguish this form of corrosion 40 from other types, and for the sake of convenience

of reference, it is herein designated as stress corrosion. Resistance to this type of corrosive attack is especially important in cases where relatively thin sheets are employed. Although the alloy without zinc rarely if ever fails in normal service even though it is under stress, yet because exceptionally severe conditions are sometimes encountered it becomes very desirable to improve the resistance to this type of attack 5 also.

The presence of 0.1 to 3 per cent zinc in the 10 alloy does not interfere with its working characteristics, nor does it disturb the responsiveness to the usual thermal treatments. The principal effect of the zinc is to increase the 15 resistance to stress corrosion. However, in order to obtain this effect, the zinc must be used in combination with cadmium, since zinc alone does not produce the improvement.

The amount of zinc which is needed to effect 20 this improvement varies between 0.1 and 3 per cent, with 1 to 2 per cent being preferred. If especially severe conditions are to be encountered, it is generally desirable to add zinc within 25 the upper portion of the foregoing ranges rather than to use smaller amounts.

Although the beneficial effect of zinc and cadmium in inhibiting stress corrosion is evident in 30 alloys containing 2 to 12 per cent copper, 0.1 to 2 per cent silicon, and 0.005 to 0.1 per cent tin, I have found that these alloy additions are especially effective in cases where these elements are present within the ranges of 2 to 6 per cent copper, 0.2 to 1 per cent silicon, and 0.03 to 0.07 per cent tin.

In order to adapt the base alloy of aluminum, copper, silicon and tin to special conditions it is frequently desirable to modify or amplify certain properties without substantially altering the fundamental characteristics. I have found it to 40 be advantageous for this purpose to add a total of from 0.01 to 1.5 per cent of one or more of the hardening elements manganese, chromium, titanium, molybdenum, boron, tungsten, vanadium, zirconium, beryllium, nickel, and cobalt. The 45 addition of these elements permits a closer control of such properties as grain size, recrystallization temperature, workability, machinability, and others. The amounts of the individual elements that may be used fall within the following 50

ranges: manganese, 0.1 to 1.5 per cent; chromium 0.1 to 1 per cent; titanium, 0.03 to 0.5 per cent; molybdenum, 0.05 to 1 per cent; boron, 0.01 to 0.5 per cent; tungsten, 0.05 to 1 per cent; vanadium, 0.05 to 1 per cent; zirconium, 0.05 to 0.5 per cent; beryllium, 0.01 to 0.5 per cent; nickel, 0.05 to 1 per cent; and cobalt, 0.05 to 1 per cent.

An illustration of the effectiveness of cadmium and zinc in improving the resistance to stress 10 corrosion is to be found in the following test results. Five alloys in the form of sheet specimens 0.064 inch in thickness were tested. The composition of the alloys was as follows:

15 *Per cent composition*

| Alloy | Copper | Manganese | Silicon | Tin  | Magnesium | Cadmium | Zinc  |
|-------|--------|-----------|---------|------|-----------|---------|-------|
| A     | 4.4    | 0.8       | 0.8     | 0.05 | 0.005     | -----   | ----- |
| B     | 4.4    | 0.8       | 0.8     | 0.05 | 0.02      | -----   | ----- |
| C     | 4.4    | 0.8       | 0.8     | 0.08 | 0.02      | 0.1     | ----- |
| D     | 4.4    | 0.8       | 0.8     | 0.08 | 0.02      | -----   | 1     |
| E     | 4.4    | 0.8       | 0.8     | 0.05 | 0.02      | 0.1     | 1     |

20 These alloys in the form of sheet were heated at 515° C. for 15 minutes, quenched in water, and aged at 160° C. for 12 hours. Specimens were cut from these sheets for mechanical property determinations, and tested. Other specimens of a shape corresponding to that of a wedge, were 25 also cut from the sheets for the stress corrosion tests. These specimens were mounted in fixtures with the base of the wedge rigidly held in position, and a load applied to the apex of the wedge normal to the plane of the specimen. The specimens thus carried a load as a cantilever beam. The load applied to each specimen was equivalent to 30 75 per cent of the yield strength of each alloy as determined by the aforesaid mechanical property tests. The stressed specimens were then 35 immersed in an aqueous 6 per cent sodium chloride solution, connected as anodes to an external source of current, and an electrical potential of 0.9 volt impressed upon them. This form of test, while much more severe than conditions encountered 40 in actual service, has been found to give in a short time a satisfactory indication of the relative resistance to stress corrosion of various aluminum base alloys. The time required for each specimen to bend, or fail to support the applied load, was noted. The average mechanical 45 properties of each alloy, and the lengths of time the various specimens supported the loads, are given in the table below.

| 55 | Alloy | Tensile strength        | Yield strength          | Elongation      | Time of failure |
|----|-------|-------------------------|-------------------------|-----------------|-----------------|
|    |       | <i>Lbs. per sq. in.</i> | <i>Lbs. per sq. in.</i> | <i>Per cent</i> | <i>Hours</i>    |
| 80 | A     | 63,770                  | 52,000                  | 10              | 10              |
|    | B     | 59,050                  | 42,100                  | 12.5            | 4.5             |
|    | C     | 66,370                  | 52,200                  | 11.8            | 4               |
|    | D     | 59,360                  | 44,400                  | 11.2            | 3               |
|    | E     | 63,940                  | 53,650                  | 9.5             | 13              |

60 Alloys A and E exhibited a pitting type of attack with scarcely any signs of intergranular corrosion, whereas alloys B, C, and D suffered from severe intergranular attack. The early failure of the latter three alloys demonstrates the effect of magnesium impurity and that the addition of zinc or cadmium alone does not materially affect the resistance to stress corrosion. The beneficial effect of zinc and cadmium when used together may be seen in alloy E. It is to be noted also that the addition of zinc and cadmium restores the alloy to the corrosion resist-

65 ant condition equal to that of the original alloy A containing magnesium within the permissible impurity range, and in some cases, there is an improvement over alloy A.

The alloys herein described are susceptible to 5 fabrication in the manner generally practiced in the art of making and shaping of aluminum base alloys. They may, furthermore, be subjected to the usual thermal treatment employed to improve the strength of aluminum base alloys. 10 This treatment generally consists in heating the alloys at an elevated temperature, above about 475° C., and rapidly cooling to ordinary or slightly elevated temperatures. This may be followed by an aging or precipitation hardening at room 15 temperature, or at any temperature up to about 200° C. The aging above room temperature is generally referred to as artificial aging and is usually applied to those alloys which do not age at room temperatures. The aluminum-silicon-copper-tin alloys are generally artificially aged in 20 order to take full advantage of the high strength which can be developed in the alloys.

The term aluminum as used hereinabove and in the appended claims denotes the metal of the 25 purity—exclusive of the magnesium impurity as herein defined—that is commercially available.

Having thus described my invention and a preferred embodiment thereof, I claim:

1. A heat treated and artificially aged aluminum base alloy containing from 2 to 12 per cent copper, 0.1 to 2 per cent silicon, 0.005 to 0.1 per cent tin, 0.005 to 0.03 per cent magnesium, 0.01 to 0.15 per cent cadmium and 0.1 to 3 per cent zinc, the balance being aluminum. 30

2. A heat treated and artificially aged aluminum base alloy containing from 2 to 12 per cent copper, 0.1 to 2 per cent silicon, 0.005 to 0.1 per cent tin, 0.005 to 0.03 per cent magnesium, 0.01 to 0.15 per cent cadmium, 0.1 to 3 per cent zinc and 0.1 to 1.5 per cent of hardening metal of the group composed of manganese 0.1 to 1.5 per cent, chromium 0.1 to 1 per cent, titanium 0.03 to 0.5 per cent, molybdenum 0.05 to 1 per cent, tungsten 0.05 to 1 per cent, vanadium 0.05 to 1 per cent, zirconium 0.05 to 0.5 per cent, beryllium 0.01 to 0.5 per cent, nickel 0.05 to 1 per cent, boron 0.01 to 0.5 per cent, the balance of the 40 alloy being aluminum. 45

3. A heat treated and artificially aged aluminum base alloy containing from 2 to 6 per cent copper, 0.2 to 1 per cent silicon, 0.03 to 0.07 per cent tin, 0.005 to 0.03 per cent magnesium, 0.01 to 0.15 per cent cadmium, and 1 to 2 per cent zinc, the balance of the alloy being aluminum. 50

4. A heat treated and artificially aged aluminum base alloy containing from 2 to 6 per cent copper, 0.2 to 1 per cent silicon, 0.03 to 0.07 per cent tin, 0.005 to 0.03 per cent magnesium, 0.01 to 0.15 per cent cadmium, 1 to 2 per cent zinc, and 0.1 to 1.5 per cent of hardening metal of the group composed of manganese, 0.1 to 1.5 per cent, chromium 0.1 to 1 per cent, titanium 0.03 to 0.5 per cent, molybdenum 0.05 to 1 per cent, tungsten 0.05 to 1 per cent, vanadium 0.05 to 1 per cent, zirconium 0.05 to 0.5 per cent, beryllium 0.01 to 0.5 per cent, nickel 0.05 to 1 per cent, boron 0.01 to 0.5 per cent, the balance of the 60 alloy being aluminum. 65

5. A heat treated and artificially aged aluminum base alloy containing from 2 to 12 per cent copper, 0.1 to 2 per cent silicon, 0.005 to 0.1 per cent tin, 0.005 to 0.03 per cent magnesium, 0.01 to 0.15 per cent cadmium and 0.1 to 3 per cent zinc, said alloy being characterized by the fact 70 75

that its resistance to stress corrosion is considerably improved over that of an aluminum base alloy containing the same amount of copper, tin, magnesium, and cadmium but without zinc.

5. A heat treated and artificially aged aluminum base alloy containing from 2 to 6 per cent copper, 0.2 to 1.5 per cent silicon, 0.1 to 1.5 per cent manganese, 0.03 to 0.07 per cent tin, 0.005 to 0.03 per cent magnesium, 0.01 to 0.15 per cent

cadmium, and 0.1 to 3 per cent zinc, and the balance of the alloy being aluminum.

7. A heat treated and artificially aged aluminum base alloy containing 4.4 per cent copper, 0.8 per cent silicon, 0.8 per cent manganese, 0.02 per cent magnesium, 0.05 per cent tin, 0.1 per cent cadmium, 1 per cent zinc, and the balance aluminum.

JOSEPH A. NOCK, JR.